

## UNITED STATES PATENT OFFICE

1,920,542

NEW DYEING PREPARATION AND ITS  
CONVERSION TO DYESTUFFS

Arthur Zitscher, Wilhelm Seidenfaden, and Karl Jellinek, Offenbach-on-the-Main, Germany, assignors to General Aniline Works, Inc., New York, N. Y., a Corporation of Delaware

No. Drawing. Application September 3, 1931,  
Serial No. 561,088, and in Germany September  
4, 1930

## 20 Claims. (Cl. 8-6)

Our present invention relates to new dyeing preparations and their conversion to dyestuffs.

These dyeing preparations contain a diazo-sulfonate of the diarylamine series corresponding to the probable general formula:



wherein X means a naphthalene nucleus or a radical of the benzene series which may contain in the para-position to the NH-group a further  $-N=N-SO_3\text{-alkali-metal}$  group, and R means a radical of the benzene series, and a combining component containing a hydroxy or a O-alkali-metal group whereof the adjacent position is capable of attaching an arylazogroup.

As substituents present in the benzene nuclei of the diazo-sulfonates may be specifically named: alkyl, alkoxy, aryloxy, alkylmercapto, aroylamino, halogen, nitro, arylsulfonyl, arylaminocarbonyl.

The diazo-sulfonates we use in our present invention are described and claimed in the co-pending U. S. application Serial No. 561,087 filed on September 3, 1931, in the name of Arthur Zitscher and Wilhelm Seidenfaden.

As combining components of the aforesaid kind may be named: 2-hydroxynaphthalene, its nuclear substitution products, as, for instance, aroylamino-hydroxynaphthalenes, (2-hydroxynaphthalene-3-carbonyl)-amino-aryls (as described in U. S. Patents Nos. 1,101,111 and 1,140,747), (6-halogen- or aroylamino-2-hydroxynaphthalene-3-carbonyl)-amino-aryls (see German Patent No. 396,519 and British Patent No. 330,349); derivatives of 1-hydroxy-naphthalene-4-carboxylic acid (see U. S. Patent No. 1,453,660), as, for instance, 1-hydroxy-naphthalene-4-phenyl-ketone; compounds containing an acidic methylene group capable of being combined with diazocompounds, as, for instance pyrazolones and derivatives of  $\beta$ -ketonaldehyde, for instance, acetoacetyl-amino-aryls and di-(aceto-acetyl-amino)-aryls (see U. S. Patent Nos. 1,594,864, 1,594,866, 1,594,867, 1,580,709, 1,634,090); dihydroxy-quinolines (see U. S. applications Serial Nos. 352,317, 352,318, 352,319; British Patent No. 332,940); (2-hydroxy-carbazole-3-carbonyl)-amino-aryls, (2-hydroxy-benzocarbazole-3-carbonyl)-amino-aryls, (2-hydroxy-anthracene-3-carbonyl)-amino-aryls.

These dyeing preparations yield, when applied in an alkaline medium to fibers, by steaming only, insoluble azodyestuffs on the fibers.

Such applying to the fibers consists in dyeing according to the one-bath-method or in print-

ing. The dyebath or the printing paste or also the powdery dyeing preparations themselves are advantageously mixed with dyeing expedients having wetting, emulsifying or dissolving properties, or also with the additional agents customary in using nitrosamine-printing-colors, as, for instance chromate. Furthermore sulfur is advantageously added to the printing paste. Thereby the quickness and the evenness of the dyestuff formation is favorably influenced.

In order to further illustrate our invention the following examples are given, the parts being by weight and all temperatures in centigrade degrees. But we wish it to be understood that we are not limited to the particular conditions or specific products mentioned therein.

## Example 1

A printing paste which contains:  
63 parts of the sodium salt of diphenylamine-4'-bisdiazo-sulfonic acid  
25 parts of (2-hydroxy-naphthalene-3-carbonyl-amino) benzene  
30 parts of caustic soda lye of 34° Bé.  
20 parts of thioglycol  
362 parts of water  
500 parts of starch tragacanth-thickening

is printed on textile materials. The goods thus printed are dried, steamed for 7 minutes in the Mather-Platt, rinsed hot and shortly soaped.

In this manner a beautiful bluish black print is obtained.

## Example 2

By using a printing paste which contains 20 parts 1-(2-hydroxy-carbazole-3-carbonyl-amino)-2-methyl-benzene, 50 parts of diphenylamine-4,4'-bis-diazosulfonate and the other ingredients of the paste used in Example 1 and by working otherwise as described above, a puce-brown print is obtained.

4,4'-di-(aceto-acetyl-amino)-3,3'-dimethyl-diphenyl yields by an analogous process a brown orange print.

## Example 3

A printing paste which contains:  
20 parts of the sodium salt of 4'-methoxy-diphenyl-amine-4-diazo-sulfonic-acid  
15 parts of (2-hydroxy-naphthalene-3-carbonyl-amino)-benzene  
20 parts of caustic soda lye of 34° Bé.  
15 parts of thioglycol  
430 parts of water  
500 parts of starch tragacanth-thickening

is printed on the materials. Then the goods are

dried, steamed for 7 minutes in the Mather-Platt, rinsed hot, soaped and rinsed again.

In this manner a clear navy-blue print is obtained.

5 Diphenyl-amine-4-diazo-sulfonate yields when used in an analogous manner a more reddish navy-blue print.

*Example 4*

10 A printing paste which contains:  
22 parts of the sodium salt of diphenyl-amine-4,4'-bis-diazo-sulfonic acid  
25 parts of 1-(2-hydroxy-naphthalene-3-carbonyl-amine)-2-methoxy-benzene  
30 parts of caustic soda lye of 34° Bé.  
15 8 parts of finely powdered sulfur  
20 parts of thioglycol  
395 parts of water  
500 parts of starch-tragacanth-thickening  
20 is printed, the goods are steamed for 5 minutes, rinsed hot and soaped. In this manner a full black print is obtained.

*Example 5*

25 A printing paste which contains:  
20 parts of the sodium salt of 4'-methoxy-diphenyl-amine-4-diazo-sulfonic-acid  
15 parts of (2-hydroxy-naphthalene-3-carbonyl-amine)-benzene  
30 20 parts of caustic soda lye of 34° Bé.  
4 parts of finely powdered sulfur  
20 parts of alcohol  
15 parts of Turkey-red-oil  
15 parts of sodium chromate solution 1:4  
35 391 parts of water  
500 parts of starch-tragacanth-thickening  
is printed. The goods are dried, steamed for 5 minutes in the Mather-Platt and finished as described above.  
40 In this manner a dark navy-blue print is obtained; by using a paste of lower concentration beautiful light blue shades are obtained.

*Example 6*

45 A bleached calico fabric is impregnated in a solution which contains:  
20 parts of the sodium salt of 4'-methoxy-diphenyl-amine-4-diazo-sulfonic-acid  
50 15 parts of (2-hydroxy-naphthalene-3-carbonyl-amine)-benzene  
20 parts of caustic potash-lye of 34° Bé.  
15 parts of alcohol  
15 parts of thioglycol  
55 15 parts of sodium-chromate solution 1:4  
50 parts of mucilage of tragacanth 65:1000  
50 parts of water  
The fabric is dried and steamed for 7-10 minutes in the Mather-Platt. Then it is rinsed hot and soaped at the boil.  
60 In this manner a blue-self-colored dyeing is obtained.

*Example 7*

A printing paste which contains:  
65 16 parts of the sodium salt of 3-methoxy-diphenyl-amine-4-diazo-sulfonic-acid  
15 parts of 1-(2-hydroxy-naphthalene-3-carbonyl-amine)-3-nitro-benzene  
30 parts of alcohol  
70 6 parts of caustic soda lye of 34° Bé.  
5 parts of thioglycol  
454 parts of water  
450 parts of starch-tragacanth-thickening  
15 parts of neutral chromate solution 1:4  
75 is printed. The goods are dried, steamed for 7

minutes in the Mather-Platt and finished as described above.

In this manner a greenish blue print is obtained.

*Example 8*

80

A mixture of:

32.0 parts of the sodium salt of 4'-methoxy-diphenyl-amine-4-diazo-sulfonic-acid  
26.3 parts of (2-hydroxy-naphthalene-3-carbonyl-amine)-benzene 85  
6.0 parts of finely ground sulfur  
8.0 parts powdered sodium hydroxide

is ground together. The mixture is made up to a printing paste. This paste is printed on the materials, which are then steamed and washed.

In this manner a clear navy blue print is obtained.

*Example 9*

95

A mixture of:  
10.6 parts of the sodium salt of 3-methoxy-diphenyl-amine-4-diazo-sulfonic-acid  
10.0 parts of 1-(2-hydroxy-naphthalene-3-carbonyl-amine)-3-nitro-benzene  
3.0 parts of sodium hydroxide 100

is ground together. The mixture is made up to a printing paste. This paste is printed on the materials, which are then steamed and washed.

In this manner a greenish blue print is obtained.

*Example 10*

105

A mixture of:  
30.0 parts of the disodium salt of diphenylamine-4,4'-bis-diazo-sulfonic acid 110  
28.6 parts of the di-sodium salt of 1-(2-hydroxy-naphthalene-3-carbonyl-amino)-3-nitro-benzene  
8.0 parts of flowers of sulfur

is ground together. The mixture is made up to a printing paste, advantageously with the addition of caustic soda lye. This paste is printed on the materials, which are then steamed and washed. In this manner a black print is obtained.

In the following table we have inserted the shades of a series of further dyeings or prints, produced in an analogous manner:

| Salt of the diazosulfonic acid of                                                                 | (2-hydroxy-naphthalene-3-carbonyl) compound of                                              | Shade                                             | 125 |
|---------------------------------------------------------------------------------------------------|---------------------------------------------------------------------------------------------|---------------------------------------------------|-----|
| 4-amino-diphenylamine<br>Do.....                                                                  | 2-amino-1-ethoxy-benzene<br>6-chloro-2-amino-1-methoxy-benzene<br>2-amino-1-phenoxy-benzene | Dark-blue<br>Navy-blue                            |     |
| Do.....                                                                                           | 1-amino-2,5-dimethoxy-benzene                                                               | Blue                                              | 130 |
| 4-amino-2'-methyl-di-phenylamine<br>Do.....                                                       | 2-amino-1-ethyl-benzene<br>2-amino-3-methoxy-naphthalene<br>2-amino-naphthalene             | Reddish navy-blue<br>Dark-violet<br>Blackish blue |     |
| 4-amino-2'-methoxy-di-phenylamine<br>Do.....                                                      | 2-amino-4-chloro-1-ethyl-benzene<br>2-ethoxy-1-amino-benzene                                | Dark-blue                                         | 135 |
| 4-amino-2'-ethoxy-di-phenylamine<br>Do.....                                                       | 2-amino-4-chloro-1-ethyl-benzene<br>2-ethoxy-1-amino-benzene                                | Dark-blue                                         |     |
| 4-amino-2'-phenoxy-di-phenylamine<br>Do.....                                                      | 3-nitro-1-amino-benzene<br>1-amino-4-ethyl-benzene                                          | Reddish navy-blue<br>Dark-blue                    | 140 |
| 4-amino-2'-chloro-di-phenylamine<br>Do.....                                                       | 1-amino-4-ethyl-benzene<br>5-chloro-2-amino-1-methoxy-benzene                               | Reddish navy-blue                                 |     |
| 4-amino-3'-methyl-di-phenylamine<br>4-amino-3'-methoxy-di-phenylamine<br>4-amino-1-methyl-benzene | 2-amino-1-methyl-benzene                                                                    | Reddish dark-blue                                 | 145 |
| 4-amino-3'-chloro-di-phenylamine<br>4-amino-4'-methyl-di-phenylamine<br>4-amino-1-methyl-benzene  | 3-amino-1-methyl-benzene<br>4-amino-1-methyl-benzene                                        | Navy-blue<br>Reddish dark-blue                    |     |

| Salt of the diazosulfonic acid of                    | (2-hydroxy-naphthalene-3-carbonyl) compound of                                            | Shade             | Salt of the diazosulfonic acid of                                                            | (2-hydroxy-naphthalene-3-carbonyl) compound of                                  | Shade                   |
|------------------------------------------------------|-------------------------------------------------------------------------------------------|-------------------|----------------------------------------------------------------------------------------------|---------------------------------------------------------------------------------|-------------------------|
| 5 4-amino-4'-methyl-diphenylamine                    | 5 - chloro - 2 - amino - 1 - methyl-benzene                                               | Reddish navy-blue | 4 - amino - 3,2' - dichloro-diphenylamine                                                    | amino-benzene.....                                                              | Dark-violet 80          |
| 4 - amino - 4' - methoxy - diphenylamine             | 2-amino-1-methoxy-benzene                                                                 | Dark-blue         | 4 - amino - 3,4' - dichloro-diphenylamine                                                    | 4-chloro - 2,5 - dimethoxy-1-amino-benzene.....                                 | Reddish violet          |
| Do.....                                              | 4 - amino - 1 - methoxy - benzene                                                         | Do.               | 4 - amino - 3',4' - dichloro-diphenylamine                                                   | 3 - methoxy - 1 - amino-benzene.....                                            | Blackish violet         |
| 10 Do.....                                           | 3 - chloro - 1 - amino - benzene                                                          | Do.               | 4 - amino - 3-methoxy-6,2' - dimethyl-4' - chloro-diphenylamine                              | 4-chloro-1-amino-benzene.....                                                   | Violet                  |
| Do.....                                              | 5 - chloro - 2 - amino - 1 - methyl-benzene                                               | Blue              | 4-amino-3-methoxy-5-chloro-4' - methoxy - diphenyl - amine                                   | 5 - chloro - 2 - methoxy - 1 - amino-benzene.....                               | Reddish violet 85       |
| Do.....                                              | 4 - chloro - 2 - methoxy - 1 - amino-benzene                                              | Dark-blue         | 4 - amino - 2' - nitro - diphenylamine                                                       | amino-benzene.....                                                              | Blackish garnet-blue    |
| Do.....                                              | 2-amino-naphthalene.....                                                                  | Reddish navy-blue | 4 - amino - 3' - chloro - 6' - nitro-diphenylamine                                           | 2,5 - dimethoxy - 1 - amino-benzene.....                                        | Brownish garnet 90      |
| 15 Do.....                                           | (4' - amino - benzoylamo-ino)-benzene                                                     | Blue              | 4 - amino - 2,5 - dimethyl - 3' - chloro - 6' - nitro - diphenylamine                        | 2 - methyl - 1 - amino - benzene.....                                           | Brownish garnet         |
| Do.....                                              | 1(4' - amino - benzoylamo-ino) - 2 - methoxy - benzene                                    | Do.               | 4 - amino - 2',4' - dinitro-diphenylamine                                                    | 1 - amino - 4 - methoxy - benzene.....                                          | Do.                     |
| Do.....                                              | 3-amino-1-acetyl-benzene.....                                                             | Greenish blue     | Do.....                                                                                      | 1 - amino - 3 - methyl - 4 - methoxy - benzene.....                             | Do.                     |
| 20 Do.....                                           | 3 - amino - 4 - methoxy - 1 - (dimethyl - aminosulfonyl)-benzene                          | Blue              | 4 - amino - 3 - methyl - 2',4' - dinitro - diphenyl - amine                                  | 1 - amino - 2 - methyl - 4 - methoxy - benzene.....                             | Bluish garnet 95        |
| Do.....                                              | 2-amino-4-ethylsulfonyl - 1 - methyl - benzene                                            | Greenish blue     | 4 - amino - 3 - methoxy - 2',4' - dinitro - diphenyl - amine                                 | 1-amino-3-nitro-benzene.....                                                    | Iron-garnet             |
| 4 - amino - 4' - ethoxy - diphenylamine              | amino-benzene.....                                                                        | Do.               | 4 - amino - 3 - chloro - 2',4' - dinitro-diphenylamine                                       | 1 - amino - 2 - methyl - benzene.....                                           | Brownish claret red 100 |
| 25 Do.....                                           | 2-amino-1-methyl-benzene                                                                  | Dark-blue         | 4 - amino - 3,2',4' - trinitro-diphenylamine                                                 | 1-amino - 2,5 - dimethoxy-benzene.....                                          | Bluish garnet           |
| Do.....                                              | 3-amino-1-methyl-benzene                                                                  | Do.               | 4 - amino - 2,5 - dimethoxy-2',4' - dinitro - diphenyl - amine                               | amino-benzene.....                                                              | Bluish black            |
| Do.....                                              | 4 - amino - 1 - methoxy - benzene                                                         | Do.               | Do.....                                                                                      | 1 - amino - 2 - methyl - 4 - methoxy-benzene.....                               | Greenish black 105      |
| Do.....                                              | 3-amino-1-chloro-benzene                                                                  | Greenish blue     | Do.....                                                                                      | 2 - amino - naphthalene.....                                                    | Do.                     |
| Do.....                                              | 3,4 - dichloro - 1 - amino - benzene                                                      | Blue              | Do.....                                                                                      | 1 - amino - 2 - ethoxy - benzene.....                                           | Blackish green          |
| 30 Do.....                                           | 2-amino-naphthalene.....                                                                  | Reddish navy-blue | Do.....                                                                                      | 1 - amino - 3 - 4 - dimethoxy-5-chloro-benzene                                  | Black                   |
| 4-amino-4'-ethoxy-diphenylamine                      | 1 (4'-amino-benzoylamo-no)-2-methyl-benzene, 1(4'-amino-benzoylamo-no) - 3-nitro-benzene. | Blue              | Do.....                                                                                      | 1 - amino - 3 - methyl - 4 - methoxy-benzene.....                               | Bluish violet 110       |
| 35 4-amino-4'-phenoxy-di-phenylamine                 | 4-amino-1 ethoxy-benzene.....                                                             | Reddish dark blue | 4-amino-3'-(phenylamino-carbonyl)-diphenylamine                                              | amino-benzene.....                                                              | Navy blue               |
| 4-amino-4'-methylmercap-to-diphenylamine             | 4-chloro-1-amino-benzene.....                                                             | Blue              | 4 - amino - 3(4' - methyl - benzene-sulfonyl)-di-phenylamine                                 | 1-amino-2-methyl-4-chloro-benzene.....                                          | Reddish blue            |
| 4-amino - 4' - chloro - diphenylamine                | 2-methoxy-1-amino-benzene                                                                 | Reddish navy-blue | Do.....                                                                                      | 1-amino-naphthalene.....                                                        | Do.                     |
| 40 4-amino - 4' - benzoylaminodiphenylamine          | 2-chloro-1-amino-benzene                                                                  | Clear blue        | Do.....                                                                                      | 1-amino-2-methyl-4-methoxy-benzene.....                                         | Reddish blue 115        |
| 4-amino-2-methyl-4'-methoxy-diphenylamine            | 2-ethoxy-1-amino-benzene                                                                  | Reddish blue      | 4-amino-3'-methyl-4'-methoxy-diphenylamine                                                   | 1-amino-3-nitro-benzene.....                                                    | Blue                    |
| Do.....                                              | 3-chloro-1-amino-benzene                                                                  | Greenish blue     | Do.....                                                                                      | 1-amino-4-methoxybenzene                                                        | Reddish dark blue       |
| Do.....                                              | 1-amino-naphthalene.....                                                                  | Blue              | Do.....                                                                                      | 1-amino-3-methyl-4-methoxy-benzene.....                                         | Navy blue               |
| 45 4-amino-3-methyl-4'-methoxy-diphenylamine         | amino-benzene                                                                             | Blue              | Do.....                                                                                      | 1-amino-4-methylbenzene.....                                                    | Reddish dark blue 120   |
| Do.....                                              | 1-amino-naphthalene.....                                                                  | Indigo-blue       | 4-amino-3-methyl-diphenylamine                                                               | 1-amino-3-nitro-benzene.....                                                    | Greenish blue           |
| Do.....                                              | 2-methyl-1-amino-benzene                                                                  | Dark blue         | Do.....                                                                                      | 1-amino-2-methyl-benzene.....                                                   | Dark blue               |
| 4-amino-3'-methyl-6'-methoxy-diphenylamine           | 3-methyl-1-amino-benzene                                                                  | Do.               | 4-amino-3-methoxy-diphenylamine                                                              | amino-benzene.....                                                              | Reddish blue            |
| 50 4-amino-3-methyl-4'-chlorodiphenylamine           | amino-benzene.....                                                                        | Reddish dark blue | Do.....                                                                                      | 1-amino-3-methoxy-benzene.....                                                  | Blue                    |
| 4-amino-2'-methyl-4'-chloro-diphenylamine            | 3-nitro-1-amino-benzene                                                                   | Deep blue         | 4-amino-4'-dimethyl-amino-diphenylamine                                                      | 1-amino-4-chloro-benzene.....                                                   | Blue                    |
| 4-amino-2'-methyl-5'-chloro-diphenylamine            | 1-amino-naphthalene.....                                                                  | Reddish navy-blue | 4-amino-4'-nitro-diphenylamine                                                               | 1-amino-2-methoxy-benzene.....                                                  | Greyish blue 125        |
| 55 4-amino-3'-methyl-6'-chloro-diphenylamine         | 4-chloro-2-methoxy-1-amino-benzene                                                        | Reddish navy-blue | 2(4'-amino-phenylamino)-naphthalene                                                          | 1-amino-2-methyl-benzene.....                                                   | Reddish black           |
| 4 - amino - 4' - 3 - chloro-diphenylamine            | 2-methyl-1-amino-benzene                                                                  | Blue-violet       | Do.....                                                                                      | 1-amino-4-methoxy-benzene                                                       | Blue                    |
| Do.....                                              | 3-nitro-1-amino-benzene                                                                   | Greenish blue     | Do.....                                                                                      | 1-amino-3-chloro-benzene.....                                                   | Reddish dark blue 130   |
| 60 4 - amino - 4' - methyl - 3'-chloro-diphenylamine | amino-benzene                                                                             | Reddish navy-blue | 4,4'-di-(2-hydroxynaphthalene-3-carbonylamino)-3,3' - dimethoxy - diphenyl                   | Do.....                                                                         | Dark violet             |
| 4 - amino - 2' - methoxy - 4'-chloro-diphenylamine   | 1 - amino - 2,5 - dimethoxy-benzene                                                       | Deep-violet       | (6-bromo - 2 - hydroxy-naphthalene-3-carbonyl-amino)-benzene                                 | 1 - amino - 3 - chloro-benzene.....                                             | Do.                     |
| 4 - amino - 3 - 2' - dimethyl-diphenylamine          | amino-benzene                                                                             | Reddish dark blue | 1 - 6 - bromo - 2 - hydroxy-naphthalene - 3 - carbonyl-amino) - 2 - methoxy-4-chloro-benzene | 2-hydroxynaphthalene.....                                                       | Corinth                 |
| 65 Do.....                                           | 2 - methoxy - 1 - amino-benzene                                                           | Do.               | 1 - hydroxy - naphthalene-4-phenylketone                                                     | 1 - hydroxy - naphthalene-4-phenylketone                                        | Corinth 135             |
| 4 - amino - 3,4' - dimethyl-diphenylamine            | 4 - chloro - 2 - methyl - 1 - amino-benzene                                               | Dark-blue         | 1 - 2 - hydroxy - anthracene-3 - carbonyl-amino) - 2 - methylbenzene                         | 1 - 2 - hydroxy - anthracene-3 - carbonyl-amino) - 2 - methylbenzene            | Bluish green            |
| 4 - amino - 3,2' - dimethoxy-diphenylamine           | 4 - chloro - 2 - methyl - 1 - amino-benzene                                               | Reddish blue      | 1 - phenyl - 3 - methyl - 5 - pyrazolone                                                     | 1 - phenyl - 3 - methyl - 5 - pyrazolone                                        | Brownish red            |
| 4 - amino - 3,4' - dimethoxy-diphenylamine           | 5 - chloro - 2 - methoxy - 1 - amino-benzene                                              | Reddish blue      | 4,4' - di-(acetoxymethyl - 3,3' - dimethyl-diphenyl)                                         | 4,4' - di-(acetoxymethyl - 3,3' - dimethyl-diphenyl)                            | Bright yellow           |
| 70 Do.....                                           | 2-amino-naphthalene                                                                       | Greenish blue     | 6,7 - benzo-2,4-dihydroxy-quinoline                                                          | 6,7 - benzo-2,4-dihydroxy-quinoline                                             | Orange brown            |
| Do.....                                              | 4 - chloro - 2 - methyl - 1 - amino-benzene                                               | Do.               | 1 - (6 - bromo - 2 - hydroxy-naphthalene-3-carbonylamino) - 2 - methoxy-benzene              | 1 - (6 - bromo - 2 - hydroxy-naphthalene-3-carbonylamino) - 2 - methoxy-benzene | Reddish dark blue 150   |
| 4 - amino - 2,4' - dimethoxy-diphenylamine           | amino-benzene                                                                             | Dark-blue         | Do.....                                                                                      | Do.....                                                                         | Reddish dark blue       |
| 4 - amino - 3,4' - dimethoxy-diphenylamine           | 4-chloro-1-amino-benzene                                                                  | Do.               | Do.....                                                                                      | Do.....                                                                         | Reddish dark blue       |

| Salt of the diazosulfonic acid of                   | (2-hydroxy-naphthalene-3-carbonyl) compound of                            | Shade         |
|-----------------------------------------------------|---------------------------------------------------------------------------|---------------|
| 5 4-amino-4'-ethoxy-diphenylamine                   | 1-(6-bromo-2-hydroxy-naphthalene-3-carbonylamino)-naphthalene             | Greenish blue |
| Do                                                  | 1,4-di-(2-hydroxy-naphthalene-3-carbonylamino)-2-methyl-5-methoxy-benzene | Navy blue     |
| Do                                                  | 4,4'-di-(2-hydroxy-naphthalene-3-carbonylamino)-benzo-phenone             | Greenish blue |
| 10 4-amino-3-methoxy-diphenylamine                  | 1-(2-hydroxy-anthracene-3-carbonyl-amino)-2-methyl-benzene                | Bluish green  |
| 15 4,4'-diamino-diphenylamine                       | 2-hydroxynaphthalene                                                      | Corinth       |
| Do                                                  | 1-(2-hydroxy-naphthalene-3-carbonylamino)-2-methyl-benzene                | Black         |
| Do                                                  | 2-(2-hydroxy-naphthalene-3-carbonylamino)-naphthalene                     | Black         |
| 20 4,4'-diamino-2-chloro-3,3'-dimethyldiphenylamine | (2-hydroxy-naphthalene-3-carbonylamino)-benzene                           | Black         |

Since an object of the present invention is to produce dyestuffs of good fastness properties which dyestuffs are insoluble in water and alkalies, it is to be understood that the aromatic nuclei of the general formulae appearing in the appended claims contain no substituents as are known to render organic compounds soluble in water or alkalies and to tend to depreciate the fastness of the dyestuffs to alkalies. Substituents of this kind are the sulfonic acid, the carboxylic acid and the hydroxy group.

35 We claim:

1. As new compositions of matter the dyeing preparations comprising a diazo-sulfonate of the diaryl-amine series corresponding to the probable general formula:



wherein X means a naphthalene nucleus or a radical of the benzene series which may contain in the para-position to the NH-group a further  $-N=N-SO_3$ -alkali-metal group and R means a radical of the benzene series and a combining component containing a hydroxy or a O-alkali-metal group whereof the adjacent position is capable of attaching an arylazo group, which dyeing preparations yield in the presence of caustic alkali by steaming azo-dyestuffs insoluble in water and alkali.

2. As new compositions of matter the dyeing preparations comprising a diazo-sulfonate of the diarylamine series corresponding to the probable general formula:



60 wherein X means a naphthalene nucleus or a radical of the benzene series which may contain in the para-position to the NH-group a further  $-N=N-SO_3$ -alkali-metal group and R means a radical of the benzene series and an azo coupling component which contains a hydroxy or a O-alkali-metal group, a free ortho-position relative to the said group capable of attaching an arylazo group and which may contain as substituents aroylamino, aroyl, arylaminocarbonyl, which dyeing preparations yield in the presence of caustic alkali by steaming azo dyestuffs insoluble in water and alkali.

75 3. As new compositions of matter the dyeing preparations comprising a diazo-sulfonate of the

diphenylamine series corresponding to the probable general formula



80

wherein the benzene nuclei may contain alkyl, alkoxy, aryloxy, halogen or nitro and Y means hydrogen or one of the aforesaid substituents or a second  $-N=N-SO_3$ -alkali-metal group and a combining component containing a hydroxy or a O-alkali-metal group whereof the adjacent position is capable of attaching an arylazo group, which dyeing preparations yield in the presence of caustic alkali by steaming azo-dyestuffs insoluble in water and alkali.

85 4. As new compositions of matter the dyeing preparations comprising a diazo-sulfonate of the diphenylamine series corresponding to the probable general formula:



90

wherein the benzene nuclei may contain alkyl, alkoxy, aryloxy, halogen or nitro and Y means hydrogen or one of the aforesaid substituents or a second  $-N=N-SO_3$ -alkali-metal group and an azo coupling component which contains a hydroxy or a O-alkali-metal group, a free ortho-position relative to the said group capable of attaching an arylazo group and which may contain 105 as substituents aroylamino, aroyl, arylaminocarbonyl, which dyeing preparations yield in the presence of caustic alkali by steaming azo-dyestuffs insoluble in water and alkali.

100 5. As new compositions of matter the dyeing preparations comprising a diazo-sulfonate of the diaryl-amine series corresponding to the probable general formula:



115

wherein X means a naphthalene nucleus or a radical of the benzene series which may contain in the para-position to the NH-group a further  $-N=N-SO_3$ -alkali-metal group and R means a radical of the benzene series, and a (2-hydroxy-120 naphthalene-3-carbonyl)-amino-aryl of the formula:



125

wherein Z means a radical of the benzene or naphthalene series, which dyeing preparations yield in the presence of caustic alkali by steaming azo-dyestuffs insoluble in water and alkali.

130

6. As new compositions of matter the dyeing preparations comprising a diazo-sulfonate of the diphenylamine series corresponding to the probable general formula:



135

wherein the benzene nuclei may contain alkyl, alkoxy, aryloxy, halogen or nitro and Y means hydrogen or one of the aforesaid substituents or a second  $-N=N-SO_3$ -alkali-metal group, and a (2-hydroxy-naphthalene-3-carbonyl)-amino-aryl of the formula:



145

wherein Z means a radical of the benzene or naphthalene series, which dyeing preparations

150

yield in the presence of caustic alkali by steaming azo-dyestuffs insoluble in water and alkali. 7. As new compositions of matter the dyeing preparations comprising a diazo-sulfonate of the 5 diphenylamine series corresponding to the probable general formula:



10 wherein the benzene nuclei may contain alkyl, alkoxy, aryloxy, halogen or nitro, and a (2-hydroxy-naphthalene-3-carbonyl)-amino-aryl of the formula:



(wherein Z means a radical of the benzene or 20 naphthalene series), which dyeing preparations yield in the presence of caustic alkali by steaming azo-dyestuffs insoluble in water and alkali.

8. As a new composition of matter the dyeing preparation consisting of

25 32, 0 parts of the sodium salt of 4'-methoxy-diphenylamine-4-diazo-sulfonic acid

26, 3 parts of (2-hydroxy-naphthalene-3-carbonyl)-amino-benzene

6 parts of finely ground sulfur

30 8 parts of powdered sodium hydroxide, which dyeing preparation yields, when brought onto fibers, by steaming clear navy blue dyeings and printings.

9. As a new composition of matter the dyeing 35 preparation consisting of

10, 6 parts of the sodium salt of 3-methoxy-diphenylamine-4-diazo-sulfonic acid

10 parts of 1-(2-hydroxy-naphthalene-3-carbonyl)-amino-3-nitro-benzene

40 3 parts of sodium hydroxide, which dyeing preparation yields, when brought onto fibers, by steaming greenish blue dyeings and printings.

10. As a new composition of matter the dyeing 45 preparation consisting of

30 parts of the disodium salt of diphenylamine-4,4'-bis-diazo-sulfonic acid

28, 6 parts of the disodium salt of 1-(2-hydroxy-naphthalene-3-carbonyl)-amino-3-nitro-benzene

50 8 parts of flowers of sulfur, which dyeing preparation yields, when brought onto fibers, by steaming black dyeings and printings.

55 11. A process which comprises applying to vegetable fibers the dyeing preparations claimed in claim 1, drying the fibers thus applied to, steaming and finishing by rinsing and soaping.

60 12. A process which comprises applying to vegetable fibers the dyeing preparations claimed in claim 2, drying the fibers thus applied to, steaming and finishing by rinsing and soaping.

65 13. A process which comprises applying to vegetable fibers the dyeing preparations claimed

in claim 3, drying the fibers thus applied to, steaming and finishing by rinsing and soaping.

14. A process which comprises applying to vegetable fibers the dyeing preparations claimed in claim 4, drying the fibers thus applied to, steaming and finishing by rinsing and soaping. 80

15. A process which comprises applying to vegetable fibers the dyeing preparations claimed in claim 5, drying the fibers thus applied to, steaming and finishing by rinsing and soaping. 85

16. A process which comprises applying to vegetable fibers the dyeing preparations claimed in claim 6, drying the fibers thus applied to, steaming and finishing by rinsing and soaping.

17. A process which comprises applying to vegetables fibers the dyeing preparations claimed in claim 7, drying the fibers thus applied to, steaming and finishing by rinsing and soaping. 90

18. A process which comprises printing vegetable fibers with a paste containing

20 parts of the sodium salt of 4'-methoxy-diphenylamine-4-diazo-sulfonic acid

15 parts of (2-hydroxy-naphthalene-3-carbonyl-amino)-benzol

20 parts of caustic soda lye of 34° Bé. 100

4 parts of finely powdered sulfur

20 parts of alcohol

15 parts of Turkey red oil

15 parts of sodium chromate solution 1:4

391 parts of water 105

500 parts of starch-tragacanth-thickening, drying the fibers thus imprinted, steaming and finishing by rinsing and soaping.

19. A process which comprises printing vegetable fibers with a paste containing

25, 6 parts of the sodium salt of 4'-methoxy-diphenylamine-4-diazo-sulfonic acid

20 parts of 1-(2-hydroxy-anthracene-3-carbonyl-amino)-2-methyl-benzene

9 parts of caustic soda lye of 34° Bé. 110

20 parts of thiodiglycol

20 parts of alcohol

405 parts of water

500 parts of starch-tragacanth-thickening, drying the fibers thus imprinted, steaming and 120 finishing by rinsing and soaping.

20. A process which comprises impregnating vegetable fibers in a bath containing

20 parts of the sodium salt of 4'-methoxy-diphenylamine-4-diazo-sulfonic acid

15 parts of (2-hydroxy-naphthalene-3-carbonyl-amino)-benzene

20 parts of caustic potash lye of 43° Bé.

15 parts of alcohol

15 parts of thiodiglycol 130

15 parts of sodium chromate solution 1:4

50 parts of mucilage of tragacanth 65:1000

50 parts of water, drying the fibers thus impregnated, steaming and 135 finishing in the usual manner.

ARTHUR ZITSCHER.  
WILHELM SEIDENFADEN.  
KARL JELLINEK.

140

CERTIFICATE OF CORRECTION.

Patent No. 1,920,542.

August 1, 1933.

ARTHUR ZITSCHER, ET AL.

It is hereby certified that error appears in the printed specification of the above numbered patent requiring correction as follows: Page 2, line 51, for "34°" read 43°; page 3, column 1, line 72, for "4-amino-2,4'-dimethoxy-" read 4-amino-2,4'-dimethoxy-; and line 144, column 5, for "Birght" read Bright; page 5, line 135, claim 20, for "in the usual manner" read by rinsing and soaping; and that the said Letters Patent should be read with these corrections therein that the same may conform to the record of the case in the Patent Office.

Signed and sealed this 28th day of November, A. D. 1933.

F. M. Hopkins

Acting Commissioner of Patents.

(Seal)